

1

3,284,199

**BUFFERED STOP BATH FOR INTERRUPTED  
PHOTOGRAPHIC DEVELOPMENT**

Vere Maffet, East Brunswick, N.J., and Earl Delzon Peters, Staten Island, N.Y., assignors to E. I. du Pont de Nemours and Company, Wilmington, Del., a corporation of Delaware

No Drawing. Filed May 2, 1963, Ser. No. 277,477  
8 Claims. (Cl. 96—50)

This invention relates to photography. Particularly it relates to a process of photographic development.

The need for an effective non-harmful means for temporarily halting the development of a photographic film has long been recognized in the trade, especially in the graphic arts field, where visual inspection of a film e.g., lithographic film, during development is an integral and critical part of development.

In practice, proper development of an ortho litho film which has been exposed imagewise to a continuous tone subject or through a halftone screen is accomplished by selection of an area of the negative to have a predetermined density or percent dot value. A certain percent dot (say 10%), means in the trade that 10% of the available space in the area selected for examination must be taken up by halftone dots. The density or percentage value of dots on a negative when processing has been completed can be determined by instrumental methods, but during development these values are estimated visually by inspection of a selected area, frequently with a magnifying glass in the case of halftone dots. A technician performing such development depends upon his judgment to provide a properly developed film. There are two points of concern to the technician, the first being to properly judge the density or percent dot in the area selected and the second to be able to judge rate of development.

The rate of development of lithographic films is characterized by an induction period of about 15 to 30 seconds during which time very little appears to be happening. After this point, development occurs rapidly and will be attained in times varying between about 1½ to 3 minutes depending upon the particular film being developed.

The need and demand for a high quality, properly developed film in the graphic arts trade does not leave even the skilled technician much latitude in development time. Most graphic arts shows require the development of their lithographic films to be stopped within  $\pm 5$  seconds of the optimum time and many shops have tighter limits such as  $\pm 2$  seconds. In such a situation, improper development time causes a loss of film and a waste of manpower. Such losses in many instances result in an average of 30 sheets of film out of every 100 not producing a satisfactory negative.

A similar problem also arises in the development of aerial cine films. The times for proper development of cine aerial films may vary between 5 and 15 minutes but the time latitude allowable to obtain a high quality negative is small. The criticality in this field of work is many times heightened, because only one exposure of the scene taken is available which makes necessary the correct development the first time.

Because of the importance of correct development in aerial photography, a solution for temporarily halting development was sought. One such solution having a pH of approximately 3 and containing a high bromide ion concentration stops development but has a number of disadvantages. First, it does not completely stop development so that, during inspection of the film, a slight amount of development occurs which is commonly called "density creep." Second, continuation of development by reinsertion of the sheet in the developer is uneven and irregular. Third, exhaustion of the developer occurs much more

2

rapidly, requiring the use of much larger volumes of developer. The use of such a solution is costly and generally impractical.

It is, therefore, an object of this invention to provide a process of development which allows the alternate halting and continuation of development of a photographic film without deleterious effects on the film or developer. A further object of this invention is to provide a process which instantaneously and evenly stops development. A still further object is to provide a process which allows even and instantaneous continuation of development following interruptions. A still further object is to provide a process which halts development and allows inspection of a film without so-called "density creep" occurring. Still further objects will be apparent from the following description of the invention.

The foregoing objects are accomplished by the process of this invention which temporarily halts the development of a photographic film, and which permits continuation of development without deleterious effects to the film or developer. The process comprises

(1) Placing an exposed photographic film containing latent silver halide images which has been partially developed, in an aqueous solution containing at least one buffering compound, said buffer solution

(a) Having a pH below that at which the developer becomes inactive,

(b) Having a buffering capacity such that the introduction of 0.10 equivalent of sodium hydroxide into 1000 milliliters of the unused buffer solution at a pH of  $7.2 \pm 0.2$  will cause a pH rise of not more than 5.0 pH units or less than 0.5 pH unit, and

(2) Reinserting the film in the developer to continue development of the film.

In practicing the above process, development of an exposed photographic film is commenced in the usual manner using the normal silver halide developer for the particular film, care being taken not to overdevelop the film. The film is removed from the developer and placed in a buffer solution having the specified characteristics. The film is agitated in the buffer solution (usually at the same temperature as the developer) for 15–20 seconds allowing time for neutralization. It is then removed for safe-light inspection. The degree of development is noted by inspection of the density or halftone dot value attained and the film is placed back in the developer for further development if desired. This cycle of halting and commencing development is continued until the desired density or halftone dot value is attained, after which the subsequent steps of fixation, etc., are carried out in the usual way.

The maximum pH specified for the buffer solution will of course depend on the pH at which the developer being used becomes inactive. The required pH limit may be selected from the inactive pH of the developers listed below:

(1) A typical general purpose developer for films, papers and plates has a working pH of approximately 9.8 and is inactive at pH=9.0 or below. Such a developer may be used for blue sensitive, orthochromatic and panchromatic sensitized silver halide films.

(2) A typical fast-acting, continuous tone developer has a working pH of approximately 9.3 and is inactive at pH=8.6 or below. Such a developer may be used for blue sensitive, orthochromatic and panchromatic sensitized silver halide films.

(3) A typical fine grain, continuous tone developer has a working pH of approximately 8.75 and is inactive at pH=8.2 or below. Such a developer may be used for blue sensitive, orthochromatic and panchromatic sensitized silver halide films.

(4) A typical developer for lithographic films has a

working pH of approximately 9.85 and is inactive at pH=9.00 or below. Such a developer is typically used for blue-sensitive and orthochromatic sensitized silver halide films.

(5) A typical metol hydroquinone developer for X-ray films has a working pH of approximately 10.75 and is inactive at pH=9.5 or below. Such a developer is typically used for products having no sensitizing dyes present.

Developers useful with the buffers described above and shown in subsequent examples will include those types used in the photographic field for development of black-and-white and color films, papers and plates. The inactive pH of other developers not covered by the above list can be determined experimentally or found in the literature.

The pH characteristics of the buffers of this invention are important to the extent that they must be below the inactive pH of the developers with which they are used, but the buffering capacity of each is still more important since it is well known that acid stop baths have a low pH but are inoperable in the process of this invention. The buffering capacity of the buffers must be (1) high enough to readily overcome the buffered pH of the developer in a sheet of film and bring it below the inactive pH of the developer when placed in the buffer solution and (2) low enough to be readily overcome by the alkalinity of the developer when development is reinitiated.

If the buffering capacity of the buffer is too low, it will be exhausted too rapidly and not allow a practicable number of sheets to be processed. On the other hand, if the buffering capacity is too high, it will exhaust the developer more rapidly than would normally occur.

Thus to determine whether a buffer is useful in the process of this invention:

(1) Select any buffer combination.

(2) Add sufficient amounts of the buffer constituents in a one liter beaker staying within the limits of solubility of the substituents. In doing so, bring the pH of a 1 liter solution to pH  $7.2 \pm 2$ .

(3) Add 0.1 equivalent of sodium hydroxide (NaOH) to the 1 liter solution. A one liter solution (prepared as in 2) which *increases* in pH by no less than 0.5 pH units and no more than 5 pH units when treated as described is suitable for the process of this invention. The

The invention is further illustrated by but is not intended to be limited by the following examples. The safelight used in the examples had a 15 watt lamp and used a Wratten Series 1-A filter. The lamp was positioned 54 inches above the light table. The 100-watt lamp used in the examples had a tungsten filament. In all examples except II, the film was exposed through an optical step-wedge whose densities varied by a factor of  $\sqrt{2}$ . The developed densities recorded were selected as resulting from exposure at a specific step falling near the middle of the density range for each set of tests.

#### Example I

Six equal film strips cut from a sheet of lithographic film having a coating weight of 50 mg. of silver/dec.<sup>2</sup> (viz., a silver bromochloride emulsion containing 20 mole percent silver bromide and 80 mole percent silver chloride) were exposed simultaneously by a 100-watt incandescent lamp under a 50-volt potential at a distance of 72 inches from the samples.

The film samples were put into a general purpose metol hydroquinone developer at the same time, with subsequent treatment as outlined in Table 1.

#### Formula of developer used:

|                              | Grams |
|------------------------------|-------|
| Metol                        | 1.0   |
| Sodium sulfite (anhydrous)   | 15.0  |
| Hydroquinone                 | 4.0   |
| Sodium carbonate (anhydrous) | 22.5  |
| Potassium bromide            | 0.6   |
| Water to make 1000 ml.       |       |

#### Formula of buffer used:

(1) 6.80 g. of potassium dihydrogen phosphate dissolved in 900 mls. of water.

(2) Sodium hydroxide is added until the pH is  $7.20 \pm .20$ .

(3) Water is added to make a total volume of 1000 ml. Under the method of this invention the above buffer has a buffering capacity corresponding to a pH change of 5.0 pH units. This solution has a throughput capacity of 1500 to 1750 sq. inches of film per liter using the film described above flashed and developed for 2½ minutes in the composition shown.

TABLE I.—USE OF BUFFER SOLUTION

| Film Sample Number | First Development (Mins.) | Buffer Solution, 20 Secs. <sup>1</sup> | Safe-light Table, 30 Secs. | Second Development (Mins.) | Fixed, Washed and Dried | Developed Density |
|--------------------|---------------------------|----------------------------------------|----------------------------|----------------------------|-------------------------|-------------------|
| 1-----             | 2                         | No-----                                | No-----                    | 0                          | Yes-----                | 1.86              |
| 2-----             | 2½                        | No-----                                | No-----                    | 0                          | Yes-----                | 2.06              |
| 3-----             | 2                         | Yes-----                               | No-----                    | 0                          | Yes-----                | 1.86              |
| 4-----             | 2                         | Yes-----                               | Yes-----                   | 0                          | Yes-----                | 1.86              |
| 5-----             | 2                         | No-----                                | Yes-----                   | 0                          | Yes-----                | 2.00              |
| 6-----             | 2                         | Yes-----                               | Yes-----                   | ½                          | Yes-----                | 2.05              |

<sup>1</sup> If an ordinary acid stop bath (approx. 1.3% acetic acid in water by volume) is substituted for the Buffer Solution, return of the film to the developer as in Step 6 above results in direct degradation of the developer by reduction of pH. Moreover, reinitiation of development occurs in a sporadic and uneven manner, giving uneven densities of unpredictable magnitude.

lower pH change limit of 0.5 pH units represent a buffer of high buffering capacity. It was found that a buffer having a smaller pH change than 0.5 pH unit would start to increase the exhaustion rate of the developer, but higher pH changes show no harmful effects to the developer.

The higher pH change limit of 5.0 represents a buffer of lower buffering capacity. Such a limit is a practical one and a buffer possessing such a buffering capacity can pass a minimum of 400 sq. inches/liter of film which has first been passed through a developer. A preferred range of pH increase for a liter of buffer solution at a pH=  $7.2 \pm 0.2$  is no less than 0.5 pH unit and no more than 2.0 pH units.

Points of particular interest illustrated by these data are noted as follows:

(a) Comparison of Samples 1 and 3 shows that immersion of the film in the buffer solution halts development instantly.

(b) Comparison of Samples 1 and 4 shows that use of the buffer solution allows inspection of the film on a safe-light table without attendant density increase.

(c) Comparison of Samples 1 and 5 illustrates the magnitude of density increase during inspection to be expected if the buffer solution treatment is not employed.

(d) Samples 1 and 2 show the density difference between 2 and 2½ minutes development.

(e) The equivalence of densities of Samples 2 and 6 shows the absence of a second induction period during

the second development, and also shows that the end result is determined by the total development time and is not influenced by the fact that there was an interruption during the development.

The foregoing discussion and description of the use of buffer solutions in controlling development has involved line exposures and a developer designed for that type exposure. Another area of great interest involving the use of lithographic films is that of halftone exposures with subsequent development in a high contrast litho developer of the hydroquinone-parafomaldehyde type or similar developers. While it is much more difficult to present quantitative data describing the formation and characteristics of halftone dots, as was done in Table I for line-exposure density relationships, it may be stated that the action and effectiveness of the buffer solution in controlling the formation of halftone dots is the same as that described and illustrated for line exposures. The following qualitative description will serve to illustrate the point.

#### Example II

Six equal film strips cut from the lithographic film of Example I and a different lithographic film having a bromochloride emulsion containing 30 mole percent silver bromide and 70 mole percent silver chloride and a coating weight of 51.5 mg. of silver/dec.<sup>2</sup> were exposed simultaneously in a manner analogous to Example I using a 100-watt incandescent lamp under 85-volt potential 72 inches from the samples. The samples of each type were exposed in contact with a magenta screen (150 lines/inch) to produce approximately a 50% dot when developed 2½ minutes at 68° F. in a typical high contrast lithographic developer. The film samples were put into the developer simultaneously, with subsequent treatment as outlined in Table II.

##### Formula of developer used:

|                              | Grams |
|------------------------------|-------|
| Metol                        | 1.5   |
| Sodium sulfite               | 22.5  |
| Hydroquinone                 | 6.0   |
| Sodium carbonate (anhydrous) | 34.0  |
| Potassium bromide            | 1.0   |
| Water to make 1000 ml.       |       |

The buffer used was the same as described in Example I.

(a) Dots on Samples 1, 3 and 4 were not detectably different from each other.

(b) Dots on Samples 2 and 6 were not detectably different from each other but were, as expected, larger than the dots on Samples 1, 3 and 4.

(c) The dots on Sample 5 were definitely larger and filled in relative to those on Samples 1, 3 and 4.

(d) The observation noted in (a) shows that treatment in the buffer solution halts growth of the halftone dots and allows inspection of the film on a safelight table without attendant dot growth.

(e) The result recorded in (b) shows the absence of a second induction period during the second development, and also shows that the end result is determined by the total development time and is not influenced by the fact that there was an interruption during the development.

(f) The dot growth indicated in (c) during inspection without prior treatment in the buffer solution is a manifestation of uncontrolled and undesirable continuation of development during the inspection period.

#### Example III

Six equal film strips cut from a sheet of X-ray film (a silver iodobromide emulsion containing 1.7% silver iodide and 98.3% silver bromide and a coating weight of 120 mg. of silver/dec.<sup>2</sup>) were exposed simultaneously by a 100-watt lamp under a 25-volt potential at a distance of 72 inches from the samples.

The film samples were put simultaneously into a typical X-ray developer with subsequent treatment as outlined in Table III.

##### Formula of developer used:

|                              | Grams |
|------------------------------|-------|
| Metol                        | 5.0   |
| Sodium sulfite (anhydrous)   | 60.0  |
| Hydroquinone                 | 7.5   |
| Sodium carbonate (anhydrous) | 50.0  |
| Potassium bromide            | 4.5   |
| Water to make 1000 ml.       |       |

##### Formula of buffer used:

(1) 80.0 gr. of boric acid crystals dissolved in 900 mls. of water.

(2) Sodium hydroxide is added until the pH=7.20±20.

(3) Water is added to make a total volume of 1000 ml.

The above formula has a buffering capacity corresponding to a pH change of 1.5 pH units when tested by the method of this invention.

TABLE III.—USE OF BUFFER SOLUTION

| Film Sample Number | First Development Time (Mins.) | Buffer Solution, 20 Secs. | Safe-light Table, 60 Secs. | Second Development Time (Mins.) | Fixed, Washed and Dried | Developed Density |
|--------------------|--------------------------------|---------------------------|----------------------------|---------------------------------|-------------------------|-------------------|
| 1                  | 3                              | No                        | No                         | 0                               | Yes                     | 1.02              |
| 2                  | 3                              | Yes                       | No                         | 0                               | Yes                     | 1.04              |
| 3                  | 3                              | Yes                       | Yes                        | 0                               | Yes                     | 1.04              |
| 4                  | 5                              | No                        | No                         | 0                               | Yes                     | 1.71              |
| 5                  | 3                              | Yes                       | No                         | 2                               | Yes                     | 1.78              |
| 6                  | 3                              | Yes                       | Yes                        | 2                               | Yes                     | 1.78              |

TABLE II.—USE OF BUFFER SOLUTION  
[Halftone exposure]

| Film Sample Number | First Development (Mins.) | Buffer Solution, 20 Secs. | Safe-light Table, 30 Secs. | Second Development (Mins.) | Fixed, Washed and Dried |
|--------------------|---------------------------|---------------------------|----------------------------|----------------------------|-------------------------|
| 1                  | 2                         | No                        | No                         | 0                          | Yes                     |
| 2                  | 2½                        | No                        | No                         | 0                          | Yes                     |
| 3                  | 2                         | Yes                       | No                         | 0                          | Yes                     |
| 4                  | 2                         | Yes                       | Yes                        | 0                          | Yes                     |
| 5                  | 2                         | No                        | Yes                        | 0                          | Yes                     |
| 6                  | 2                         | Yes                       | Yes                        | ½                          | Yes                     |

Based on inspection of the halftone dots at magnification 10X and 100X, the following observations and conclusions apply to each film type:

The results here parallel those described in points (a) through (e) in Example I. Further, this example illustrates the use of a second buffer within the designated range specified by the invention besides demonstrating the workability of the process on X-ray films.

#### Example IV

Six equal film strips from a paper product (a silver iodochlorobromide emulsion containing 3.6 mole percent silver iodide, 16.4 mole percent silver chloride and 80 mole percent silver bromide and having a coating weight of 22.4 mg. of silver/dec.<sup>2</sup>) for making prints of film negatives were exposed simultaneously through a

step wedge by a 100-watt lamp under a 50-volt potential at a distance of 72 inches from the samples.

The film samples were simultaneously put into a general purpose metol hydroquinone developer as described in Example I with subsequent treatment as outlined in Table IV.

The buffer used was the same as that described in Example III.

TABLE IV.—USE OF BUFFER SOLUTION

| Film Sample Number | First Development (Mins.) | Buffer Solution, 20 Secs. | Safe-light Table, 60 Secs. | Second Development (Mins.) | Fixed, Washed and Dried | Developed Density <sup>1</sup> |
|--------------------|---------------------------|---------------------------|----------------------------|----------------------------|-------------------------|--------------------------------|
| 1                  | 1                         | No-----                   | No-----                    | 0                          | Yes-----                | 1.09                           |
| 2                  | 1                         | Yes-----                  | No-----                    | 0                          | Yes-----                | 1.10                           |
| 3                  | 1                         | Yes-----                  | Yes-----                   | 0                          | Yes-----                | 1.08                           |
| 4                  | 2                         | No-----                   | No-----                    | 0                          | Yes-----                | 1.69                           |
| 5                  | 1                         | Yes-----                  | No-----                    | 1                          | Yes-----                | 1.70                           |
| 6                  | 1                         | Yes-----                  | Yes-----                   | 1                          | Yes-----                | 1.67                           |

<sup>1</sup> At a specific step of the wedge exposure.

The above results parallel those described in points (a) through (e) in Example I and demonstrate the workability of the process on a paper product.

#### Example V

**Test.**—A high contrast paraformaldehyde-hydroquinone type developer was prepared and 1,000 milliliter portions were placed in each of two trays. Exposed sheets of lithographic film of the type described in Example I were successively developed in each developer and handled as specified.

(1) The sheets from developer No. 1 were immediately fixed and washed in the usual fashion.

(2) Each sheet from developer No. 2 was immersed in the buffer solution for 30 seconds, with agitation, and then returned to the developer. The two development periods in developer No. 2 were made equal in total time to the single development time period in developer No. 1. Following the second development period, the sheets were fixed and washed.

**Results.**—Measured as the rate of fall in density of the processed film as the test proceeded, the exhaustion rates of the two developers were identical, within the limits of reproducibility, to the exhaustion rates of two developers without the use of an intervening buffer solution.

**Conclusion.**—Return of a film to the developer after treatment in the buffer solution has no deleterious effect on the developer. The above example used the buffer described in Example III.

#### Example VI

**Test.**—A sheet of lithographic film of the type described in Example I was exposed through a step wedge and then cut into strips which were developed in a high contrast paraformaldehyde-hydroquinone type developer and then treated as follows.

(1) Strip No. 1 was immediately fixed and washed in the usual fashion.

Strips 2 through 11 were immersed in the buffer solution (buffer solution described in Example III) and then handled as specified.

Strips 2 through 6 were removed from the buffer solution after 30 seconds and hung in air in darkness. Strips 7 through 11 were left in the buffer solution.

(2) Strip No. 2 was fixed and washed after 5 minutes.

(3) Strip No. 3 was fixed and washed after 30 minutes.

(4) Strip No. 4 was fixed and washed after 1 hour.

(5) Strip No. 5 was fixed and washed after 2 hours.

(6) Strip No. 6 was fixed and washed after 4 hours.

(7) Strip No. 7 was removed from the buffer solution after 1 hour and fixed and washed.

(8) Strip No. 8 was removed from the buffer solution after 30 minutes and fixed and washed.

(9) Strip No. 9 was removed from the buffer solution after 1 hours and fixed and washed.

(10) Strip No. 10 was removed from the buffer solution after 2 hours and fixed and washed.

(11) Strip No. 11 was removed from the buffer solution after 4 hours and fixed and washed.

**Results.**—Densities were equal on all the test strips.

**Conclusion.**—There is no practical limitation on how

long films may be left in the buffer solution, nor on how long development of the film is interrupted after removal from the buffer solution. It is noteworthy that film samples 3 through 6 were dry before the end of the period of exposure to air.

Suitable emulsions for operation with the process of this invention are silver chlorobromide, silver iodobromide and silver iodochlorobromide. In addition to mixed silver halides, the silver halides used may be pure silver halides e.g. silver bromide, silver chloride.

In place of gelatin, other natural or synthetic water-permeable, organic colloid, binding agents can be used. Such agents include water permeable or water soluble polyvinyl alcohol and its derivatives, e.g., partially hydrolyzed polyvinyl acetates, polyvinyl ethers, and acetals containing a large number of extralinear —CH<sub>2</sub>CHOH— groups: hydrolyzed interpolymers of vinyl acetate and unsaturated addition polymerizable compounds such as maleic anhydride, acrylic and methacrylic acid ethyl esters, and styrene. Suitable colloids of the last mentioned type are disclosed in U.S. Patents 2,276,322, 2,276,323, and 2,397,866. The useful polyvinyl acetals include polyvinyl acetaldehyde acetal, polyvinyl butyraldehyde acetal and polyvinyl sodium o-sulfonylbenzaldehyde acetal. Other useful colloid binding agents include the poly-N-vinylactams of Bolton U.S. Patent 2,495,918, the hydrophilic copolymers of N-acrylamido alkyl betaines described in Shacklett U.S. Patent 2,833,650, and hydrophilic cellulose ether and esters.

The emulsions can contain known antifoggants, e.g., 6-nitrobenzimidazole, benzotriazole, triazaindenes, etc., as well as the usual hardeners, i.e., chrome alum, formaldehyde, dimethylol urea, mucochloric acid, etc. Other emulsion adjuvants that may be added comprise sensitizers, matting agents, plasticizers, toners, optical brightening agents, etc.

The emulsions may be coated on any suitable support, e.g., cellulose esters, cellulose mixed esters; superpolymers, e.g., polyvinyl chloride covinyl acetate; polyvinyl acetals, e.g., formals, acetals, butyral; polystyrene, polyamide, e.g., polyhexamethylene adipamide; polyesters, e.g., polycarbonates, polyethylene terephthalates, polyethylene terephthalate/isophthalate, esters formed by condensing terephthalic acid and dimethyl terephthalate with propylene glycol, diethylene glycol, tetramethylene glycol or cyclohexane-1,4 - dimethanol(hexahydro-p-xylene alcohol); paper and glass.

Suitable developers for the process of this invention are the alkaline developers which include polyphenolic developers e.g., hydroquinone, pyrogallol, pyrocatechol, 2,3-dichlorohydroquinone; aminophenols e.g., p-aminophenol, metol, 2,4-diaminophenol; polyamines e.g., p-phenylenediamine, p - diethylaminoaniline, n -  $\beta$  - methyl sulfonamidoethyl-4-aminoaniline; heterocyclic bases e.g.,

p-dihydroxyquinoline, amino and hydroxymorpholines, 1-phenyl-3-pyrazolidone etc. Combinations of such developers known to the art and with special adjuvants such as ascorbic acid may be used. The normal additions to developers can be used in all the known combinations e.g., alkalies such as lithium, sodium and potassium hydroxides, carbonates, alkylamines, and alkanolamines; borax; sodium metaborate; sodium sulfite; alkali halides e.g., bromide, chloride etc.; surface active agents e.g., polyalkyleneoxide; condensation products e.g., polyglycols, and their ethers and esters; antifoggants e.g., benzotriazole, 6-nitrobenzimidazole; hardeners e.g., formaldehyde, alum, glyoxal, glutaraldehyde; image color modifiers e.g., mercaptotetrazoles; alcohols; sequestering agents e.g., the trisodium salt of ethylene diamine tetracetic acid.

Buffers suitable for the process of this invention are those meeting the buffering capacity requirements previously specified for one liter of the buffering solution. Namely, that the addition of a 0.1 of an equivalent of sodium hydroxide to the buffer solution at a pH of 7.2 causes a rise in pH not less than 0.5 pH unit nor greater than 5 pH units. Buffers having such a buffering capacity are the

*Potassium dihydrogen phosphate/sodium hydroxide buffer system* which has a buffering capacity corresponding to a change of 5 pH units and has the following composition:

(a) Potassium dihydrogen phosphate—6.80 g. dissolved in 900 mls. of water.

(b) Sodium hydroxide added to bring the pH to 7.20  $\pm .20$ .

(c) Water added to make 1000 mls. of solution.

*Sodium monohydrogen phosphate/citric acid buffer system* which has a buffering capacity corresponding to a change of 4.3 pH units and has the following composition:

(a) Sodium monohydrogen phosphate—17.9 g. dissolved in 900 mls. of water.

(b) Citric acid added to bring the pH to 7.20  $\pm .20$ .

(c) Water added to make 1000 mls. of solution.

The process of this invention has been found to be highly advantageous in the graphic arts field where it can practically eliminate re-runs of lithographic exposures due to improper development times. The buffer used in the process of this invention stops development promptly and permits development to be re-initiated uniformly thus allowing judgment of development based on time in the developer only without giving rise to "density creep." Reinitiation of development using such buffers does not involve a second induction period which would lead to unpredictable densities.

The discussion thus far has implied uniform control of development over an entire sheet of film. In addition to this highly useful processing aid, it is also possible to employ the buffer solution in a manner somewhat analogous to that of dodging. For example, if a buffer-treated film is under inspection on a safelight table, it may be that only a selected area will be seen to require further development. Such development of localized areas, on either line or halftone exposures, may be readily accomplished by applying to the area in question a cotton swab wetted with developer. Redevelopment will be initiated immediately, and may be terminated when

desired by applying another cotton swab wetted with the buffer solution. This aspect of the development control technique offers many possibilities to processing operators. Still additional advantages will be apparent to those skilled in the art of photographic development.

We claim:

1. A process for controlling the development of a photographic film which comprises:

(1) placing an exposed photographic film containing latent silver halide images which has been partially developed, in an aqueous solution containing at least one buffering compound, said buffer solution

(a) having a pH below that at which the developer becomes inactive,

(b) having a buffering capacity such that the introduction of 0.10 equivalent of sodium hydroxide into 1000 milliliters of the unused buffer solution at a pH of  $7.2 \pm 0.2$  will cause a pH rise of not more than 5.0 pH units or less than 0.5 pH unit, and

(2) reinserting the film in the developer to continue development of the film.

2. A process according to claim 1 wherein steps (1) and (2) are repeated until the desired density is attained.

3. A process according to claim 1 wherein steps (1) and (2) are repeated until the desired silver density is attained and

(3) the developed film is then fixed.

4. A process according to claim 1 wherein the buffer solution contains potassium dihydrogen phosphate and caustic soda.

5. A process according to claim 1 wherein the buffer solution contains sodium monohydrogen phosphate and citric acid.

6. A process according to claim 1 wherein the buffer solution contains boric acid and sodium hydroxide.

7. A process according to claim 1 wherein hydroquinone is used as the sole developing agent.

8. A process according to claim 1 wherein the developer is a metol-hydroquinone developer.

#### References Cited by the Examiner

##### UNITED STATES PATENTS

45 2,280,721 4/1942 Schilling et al. ----- 96—62 X  
2,541,865 2/1951 Friedman ----- 96—63 X

##### OTHER REFERENCES

50 Luppo, Cramer, Photo. Korr., volume 52, 1915, pages 35 to 36.

Wall et al., Photographic Facts and Formulas, Boston, American Photographic Publishing Co., 1947, page 160.

Washburn, Ed., International Critical Tables, New York, McGraw-Hill, 1926, volume 1, pages 82—83.

#### References Cited by the Applicant

##### UNITED STATES PATENTS

2,184,053 12/1939 Muehler.  
2,239,284 4/1941 Draisbach.  
2,343,696 3/1944 Muehler et al.  
2,541,470 2/1951 Henn et al.

NORMAN G. TORCHIN, Primary Examiner.

C. E. Davis, Assistant Examiner.